# EUROPEAN PATENT SPECIFICATION

(11) **EP 2 260 552 B1**
(45) Date of publication and mention of the grant of the patent: **24.07.2013**
(21) Application number: 09727243.9
(22) Date of filing: 24.03.2009
(51) Int. Cl.: H01T 19/00

(54) **CORONA ROLLER COMPRISING A CYLINDRICAL BASE BODY AND A DIELECTRIC ROLLER COVER, AND METHOD FOR PRODUCING SUCH A CORONA ROLLER**
KORONAWALZE MIT ZYLINDERFÖRMIGEM GRUNDKÖRPER UND DIELEKTRISCHEM WALZENÜBERZUG SOWIE VERFAHREN ZUR HERSTELLUNG EINER DERARTIGEN KORONAWALZE
ROULEAU À EFFET DE COURONNE COMPRENANT UN CORPS DE BASE CYLINDRIQUE ET UN REVÊTEMENT DE ROULEAU DIÉLECTRIQUE AINSI QUE SUR UN PROCÉDÉ DE FABRICATION D'UN TEL ROULEAU À EFFET DE COURONNE

(30) Priority: 02.04.2008 DE 102008016851
(43) Date of publication of application: 15.12.2010
(73) Proprietor: Coatec Gesellschaft Für Oberflächenveredelung Mbh, 36381 Schlüchtern (DE)
(72) Inventor: HEUSER, Claus, 63755 Alzenau (DE); KIRST, Markus, 64572 Büttelborn (DE); JOHNER, Gerhard, 63751 Gelnhausen (DE); DUDAZY, Christian, 63486 Bruchköbel (DE)
(74) Representative: Schwan - Schwan - Schorer
(86) International application number: PCT/EP2009/053448
(87) International publication number: WO 2009/121756

(56) References cited:
- WO-A-83/01021
- US-A- 4 940 894

## Description

The invention relates to a corona roller comprising a cylindrical base body and a roller cover of dielectric material. The invention further relates to methods for producing such a corona roller.

Frequently, aluminum oxide is used as dielectric material for the roller cover of a corona roller, wherein the aluminum oxide is applied on the roller body by plasma spraying. Such rollers are used in corona systems (reference is made to the attached drawing) in which e.g. foils of plastic material are pretreated with specific electrical discharges such that oxidation processes cause the surfaces thereof to become hydrophilic and thereby can be used in printing with conventional offset processes. In view of the fact that these dielectrically effective layers of aluminum oxide frequently are porous, they are sealed with synthetic resins, and in the case that this sealing is to be effective not only superficially but rather throughout the entire thickness of the layer, this process is carried out in a vacuum, as is known from DE 199 57 644 A1 and WO 01/40544 A1. In practice, however, it turned out that even a pore-deep sealing of the aluminum oxide layer with a synthetic resin can not guarantee that no electrical breakdown to the roller core will occur. The reasons therefor are based on the one hand on the adhesion-promoting layer which usually is provided for in plasma spraying and which has a substantial topography combined with a corresponding peak action (local increase of the field strength up to an electrical breakdown - principle of a lightning conductor), and on the other hand on the dynamics of the roller body during operation including deflections, oscillations and so on, with the consequence that also the aluminum oxide layer sealed with synthetic resin will get fissures or cracks through which the electrical breakdown will take place. An electrical breakdown usually not only means an interruption of the process, but also a destruction of the functionality of the corona roller.

The object of the invention therefore is to provide for a corona roller having an increased operational safety against electrical breakdowns, and to provide for a reliable method for producing such a corona roller.

The object basic to the invention is solved by the methods claimed in claims 1 and 5 and by a corona roller according to claim 10.

The corona roller comprises a cylindrical base body and a roller cover of dielectric material. In conformity with the invention, the roller cover includes a layer of thermoplastic material applied onto the outer surface of the base body, wherein solid powder particles having electrically insulating characteristics are embedded into the material matrix of the layer in the vicinity of the surface thereof in a form-locking manner such that merely a partial region of the particles protrudes from the inner layer; and a hard, wear- and corrosion- resistant outer layer is formed at the outer side of the layer of thermoplastic material, into which the particle partial regions protruding from said layer of plastic material are embedded, with the hard, wear- and corrosion- resistant surface likewise having electrically insulating characteristics.

The cover provided for in conformity with the invention is advantageous particularly in that on the one hand no metallic adhesion-promoting layers are required thereby eliminating the risk of electrical breakdowns via the peak action due to the topography, and that on the other hand even a formation of fissures or cracks in the electrically insulating outer layer will not result in a local total breakdown of the dielectric characteristics and thus an electrical breakdown. The electrical insulation effect of the thermoplastic material, particularly when the specific resistance thereof is at least 10¹² Ω×m, is fully sufficient to secure the functioning of the corona roller, so that the outer layer disposed thereon represents an additional electrical insulation, the main function of the outer layer, however, being protection against wear. A further advantage of the coating in conformity with the invention resides in the fact that the cover of thermoplastic material having a high dielectricity also is highly chemically resistant and safely protects the roller body against corrosion. Subsurface corrosion accompanied by local delamination of the aluminum oxide layer occurs in conventional corona rollers when the surface thereof is treated e.g. with heavily acidic cleaning agents and when the roller body consists of low-alloyed steel.

The layer of plastic material particularly may be covered by an electrically insulating, wear-resistant outer functional layer into which the particle partial regions protruding from the layer of plastic material are imbedded, the outer functional layer preferably consisting of oxide ceramic, particularly Al₂O₃, Cr₂O₃, SiO2, ZrO₂ or mullite or of a mixture of two or more of these materials.

The material of the layer of plastic material particularly may be thermoplastic polyamides such as the materials known under the trade names RILSAN®, NYLON and PERSON®, i.e. polyamides on the base of castor oil and PA 11 on the base of lactame, polyamides of PA 4, PA 11 (NYLON) or polyamides of PA 6 (PERLON®).

According to a further embodiment of the invention the functional layer has a thickness from 0.05 mm to 3.0 mm, and preferably a thickness of about 0.5 mm. Whereas conventional corona rollers frequently are provided with layers of aluminum oxide which have a thickness of up to 2 millimeters and more and which are correspondingly susceptible to fissures or cracks, the cover according to the subject invention normally permits a reduction of the thickness of the oxide ceramic layer to few tenths of a millimeter. This not only has economical advantages in the production of such coatings for corona rollers, but also offers a substantially increased operational safety because layers of oxide ceramic are much less tending to the formation of cracks under dynamic loads.

A thickness from 0.5 mm to 4 mm and preferably from about 1 mm to 2 mm turned out to be particularly suited for the layer of plastic material, and the surface of the roller cover preferably has a surface roughness of 0.5 µm < Rz <500 µm, particularly a surface roughness Rz from 1.5 µm to 20 µm.

In conformity with the invention the method for producing a corona roller comprising a cylindrical base body and a roller cover of dielectric material includes a first step in which a layer of thermoplastic material is applied onto the outer surface of the base body. In a further step the layer of plastic material is heated to a viscosity similar to that of honey. Subsequently, solid (powder) particles having electrically insulating characteristics are imbedded into the material matrix of the thus heated layer of plastic material in the vicinity of the surface thereof in a form-locking manner such that merely a partial region of these particles protrudes from the inner layer. The thus prepared layer of plastic material is covered by an electrically insulating, wear-resistant outer functional layer into which the particle partial regions protruding from the layer of plastic material are embedded.

The functional layer preferably is produced by thermal spraying, wherein the first powder particles are shot into the material matrix of the heated layer of plastic material in the vicinity of the surface thereof in such a manner that they still protrude with a partial region thereof from the layer of plastic material, and wherein in the further course of the spraying operation the protruding powder particles are caused to be bonded with subsequent powder particles forming said functional layer.

According to a modified method for producing a corona roller comprising a cylindrical base body and a roller cover of dielectric material, again a layer of thermoplastic material is applied onto the outer surface of the base body and is heated to a viscosity similar to that of honey. Then particles of solid material having electrically insulating characteristics are dispersed into the material matrix of the thus heated layer of plastic material in the vicinity of the surface thereof, and a hard, wear- and corrosion resistant surface is produced by subsequently grinding the coating of thermoplastic material which in the vicinity of the surface thereof is dispersed with particles of solid material.

It is to be understood that in both embodiments of the method the outer coating additionally may be provided with a sealing which closes any pores, as known from DE 199 57 644 A1 und WO 01/40544 A1.

The single Figure shows an example of a corona roller of the above described type which consists of a roller base body 10 and a roller cover (dielectric) 11 and which is being used in a corona system. The corona system includes an electrode unit 13 provided with an extractor. A foil 12 of plastic material is supported on the corona roller which rotates in the direction of the arrow, whilst the foil passes beneath the electrode unit 13 and is pretreated by electrical discharges such that its surface becomes hydrophilic due to oxidations processes, and thus is made suitable for printing in a conventional offset process.

## Claims

1. Method for producing a corona roller comprising a cylindrical base body and a roller cover of dielectric material, wherein a layer of thermoplastic material is applied onto the outer surface of the base body, wherein the layer of plastic material is heated to a viscosity similar to that of honey, and wherein solid powder particles having electrically insulating characteristics are imbedded into the material matrix of the thus heated layer of plastic material in the vicinity of the surface thereof in a form-locking manner such that merely a partial region of said particles protrudes from said inner layer, and wherein the thus prepared layer of plastic material is covered by an electrically insulating, wear-resistant outer functional layer into which the particle partial regions protruding from said layer of plastic material are imbedded.

2. Method as claimed in claim 1, wherein the particles are shot into the material matrix of the thus heated layer of plastic material in the vicinity of the surface thereof.

3. Method as claimed in claim 1 or 2, wherein in a step of a thermal spraying operation for producing the functional layer, the first powder particles are shot into the material matrix of the heated layer of plastic material in the vicinity of the surface thereof in such a manner that they still protrude with a partial region thereof from said layer of plastic material, and wherein in the further course of the spraying operation the protruding powder particles are caused to be bonded with subsequent powder particles forming said functional layer.

4. Method as claimed in any one of the preceding claims, wherein said outer functional layer is produced at a thickness from 0.05 mm to 3.0 mm, and preferably a thickness of about 0.5 mm.

5. Method for producing a corona roller comprising a cylindrical base body and a roller cover of dielectric material, wherein a layer of thermoplastic material is applied onto the outer surface of the base body, wherein the layer of plastic material is heated to a viscosity similar to that of honey, wherein particles of solid material having electrically insulating characteristics are dispersed into the material matrix of the thus heated layer of plastic material in the vicinity of the surface thereof, and wherein a hard, wear- and corrosion resistant surface is produced by subsequently grinding the cover of thermoplastic material which in the vicinity of the surface thereof is dispersed with particles of solid material.

6. Method as claimed in claim 5, wherein the particles of solid material are dispersed into the material matrix of the thus heated layer of plastic material in the vicinity of the surface thereof by means of a sand blasting or calender system.

7. Method as claimed in any one of the preceding claims, wherein said layer of plastic material is applied onto the base body of the roller by a fluidized bed process or a thermal spray process.

8. Method as claimed in any one of the preceding claims, wherein said layer of plastic material is applied at a thickness from 0.5 mm to 4 mm.

9. Method as claimed in any one of the preceding claims, wherein the surface of the roller cover is ground or polished to a surface roughness of 0.5 µm < Rz <500 µm, particularly a surface roughness Rz from 1.5 µm to 20 µm.

10. Corona roller comprising a cylindrical base body and a roller cover of dielectric material, **characterized in that** the roller cover includes a layer of thermoplastic material applied onto the outer surface of the base body, wherein solid powder particles having electrically insulating characteristics are embedded into the material matrix of said layer in the vicinity of the surface thereof in a form-locking manner such that merely a partial region of said particles protrudes from said inner layer, and that a hard, wear- and corrosion- resistant outer functional layer is formed at the outer side of said layer of thermoplastic material, into which the particle partial regions protruding from said layer of plastic material are imbedded, said hard, wear- and corrosion- resistant outer functional layer likewise having electrically insulating characteristics.

11. Corona roller as claimed in claim 10, **characterized in that** the functional layer consists of oxide ceramic, particularly Al₂O₃, Cr₂O₃, SiO₂, ZrO₂ or mullite or of a mixture of two or more of said materials.

12. Corona roller as claimed in claims 10 or 11, **characterized in that** the thermoplastic material has a specific resistance of at least 10¹² Ω × m and/or consists of polyamide.

13. Corona roller as claimed in any one of claims 10 to 12, **characterized in that** the particles imbedded into the material matrix of the layer of plastic material in the vicinity of the surface thereof consist of the same material as the functional layer.

14. Corona roller as claimed in any one of claims 10 to 113, **characterized in that** the layer of plastic material has a thickness from 0.5 mum to 4 mm and/or the functional layer has a thickness from 0.05 mm to 3.0 mm and preferably of about 0.5 mm.

15. Corona roller as claimed in any one of claims 10 to 14, **characterized in that** the surface of the roller cover has a surface roughness of 0.5 µm < Rz <500 µm, particularly a surface roughness Rz from 1.5 µm to 20 µm.

## Patentansprüche

1. Verfahren zum Herstellen einer Koronawalze mit einem zylindrischen Grundkörper und einem Walzenbezug aus dielektrischem Werkstoff, bei dem auf die Außenfläche des Grundkörpers eine Schicht aus thermoplastischem Kunststoff aufgebracht wird, wobei die Kunststoffschicht bis zu einer honigähnlichen Viskosität erwärmt wird, und bei dem in die oberflächennahe Werkstoffmatrix der so erwärmten Kunststoffschicht Feststoffpulverpartikel mit elektrisch isolierenden Eigenschaften formschlüssig haftend derart eingebettet werden, dass nur ein Teilbereich dieser Partikel aus der Innenschicht herausragt, und bei dem die derart vorbereitete Kunststoffschicht mit einer elektrisch isolierenden, verschleißfesten äußeren Funktionsschicht beschichtet wird, in welche die aus der Kunststoffschicht herausragenden Partikel-Teilbereiche eingelagert werden.

2. Verfahren nach Anspruch 1, bei dem die Partikel in die oberflächennahe Werkstoffmatrix der erwärmten Kunststoffschicht eingeschossen werden.

3. Verfahren nach Anspruch 1 oder 2, bei dem im Zuge eines die Funktionsschicht erzeugenden thermisches Spritzvorgangs die ersten Pulverpartikel in die oberflächennahe Werkstoffmatrix der erwärmten Kunststoffschicht so eingeschossen werden, dass sie mit einem Teilbereich noch aus der Kunststoffschicht herausragen, und bei dem im weiteren Verlauf des Spritzvorgangs eine Verbindung der herausragenden Pulverpartikel mit nachfolgenden, die Funktionsschicht bildenden Pulverpartikeln bewirkt wird.

4. Verfahren nach einem der vorhergehenden Ansprüche, bei dem die äußere Funktionsschicht in einer Dicke von 0,05 mm bis 3,0 mm, vorzugsweise etwa 0,5 mm, ausgebildet wird.

5. Verfahren zum Herstellen einer Koronawalze mit einem zylindrischen Grundkörper und einem Walzenbezug aus dielektrischem Werkstoff, bei dem auf die Außenfläche des Grundkörpers eine Schicht aus thermoplastischem Kunststoff aufgebracht wird, bei dem die Kunststoffschicht bis zu einer honigähnlichen Viskosität erwärmt wird, bei dem in die oberflächennahe Werkstoffmatrix der so erwärmten Kunststoffschicht Feststoffpartikel mit elektrisch isolierenden Eigenschaften eindispergiert werden und bei dem durch anschließendes Schleifen des derart oberflächennah mit Feststoffpartikeln dispergierten thermoplastischen Kunststoffüberzugs eine harte, verschleiß- und korrosionsbeständige Oberfläche ausgebildet wird.

6. Verfahren nach Anspruch 5, bei dem die Feststoffpartikel mittels einer Sandstrahl- oder Kalanderanlage in die oberflächennahe Werkstoffmatrix der erwärmten Kunststoffschicht eindispergiert werden.

7. Verfahren nach einem der vorhergehenden Ansprüche, bei dem die Kunststoffschicht auf den Walzen-Grundkörper im Fluidized-Bed-Verfahren oder durch ein thermisches Spritzverfahren aufgetragen wird.

8. Verfahren nach einem der vorhergehenden Ansprüche, bei dem die Kunststoffschicht in einer Dicke von 0,5 mm bis 4 mm aufgetragen wird.

9. Verfahren nach einem der vorhergehenden Ansprüche, bei dem die Oberfläche des Walzenbezugs auf eine Oberflächenrauhigkeit zwischen 0,5 µm < Rz < 500 µm, insbesondere auf Rz = 1,5 µm bis 20 µm, geschliffen oder poliert wird.

10. Koronawalze mit einem zylindrischen Grundkörper und einem Walzenbezug aus dielektrischem Werkstoff, **dadurch gekennzeichnet, dass** der Walzenbezug eine auf die Außenfläche des Grundkörpers aufgebrachte Schicht aus thermoplastischem Kunststoff aufweist, in deren oberflächennahe Werkstoffmatrix Feststoffpulverpartikel mit elektrisch isolierenden Eigenschaften formschlüssig haftend derart eingebettet sind, dass nur ein Teilbereich dieser Partikel aus der Innenschicht herausragt, und dass an der Außenseite der Kunststoffschicht eine harte, verschleiß- und korrosionsbeständige Oberfläche ausgebildet ist, in welche die aus der Kunststoffschicht herausragenden Partikel-Teilbereiche eingelagert sind, und die gleichfalls elektrisch isolierende Eigenschaften hat.

11. Koronawalze nach Anspruch 10, **dadurch gekennzeichnet, dass** die Funktionsschicht aus Oxidkeramik, insbesondere Al₂O₃, Cr₂O₃, SiO₂, ZrO₂ oder Mullit oder aus einer Mischung aus zwei oder mehr dieser Werkstoffe, besteht.

12. Koronawalze nach Anspruch 10 oder 11, **dadurch gekennzeichnet, dass** der thermoplastische Kunststoff einen spezifischen Widerstand von mindestens 10¹² Ω x m hat und / oder die Kunststoffschicht aus Polyamid besteht.

13. Koronawalze nach einem der vorhergehenden Ansprüche 10 bis 12, **dadurch gekennzeichnet, dass** die in die oberflächennahe Werkstoffmatrix der Kunststoffschicht eingebetteten Partikel aus dem gleichen Werkstoff wie die Funktionsschicht bestehen.

14. Koronawalze nach einem der vorhergehenden Ansprüche 10 bis 13, **dadurch gekennzeichnet, dass** die Kunststoffschicht eine Dicke von 0,5 mm bis 4 mm aufweist und / oder dass die Funktionsschicht eine Dicke von 0,05 mm bis 3,0 mm, vorzugsweise etwa 0,5 mm, aufweist.

15. Koronawalze nach einem der vorhergehenden Ansprüche 10 bis 14, **dadurch gekennzeichnet, dass** die Oberfläche des Walzenbezugs eine Oberflächenrauhigkeit hat, die zwischen 0,5 µm < Rz < 500 µm, insbesondere bei Rz = 1,5 µm bis 20 µm, liegt.

## Revendications

1. Procédé pour produire un cylindre corona comprenant un corps de base cylindrique et un élément de recouvrement de cylindre en un matériau diélectrique, dans lequel une couche de matière thermoplastique est appliquée sur la surface extérieure du corps de base, dans lequel la couche de matière plastique est chauffée à une viscosité similaire à celle du miel, et dans lequel des particules de poudre solide ayant des caractéristiques d'isolement électrique sont intégrées dans la matrice de matériau de la couche de matière plastique ainsi chauffée au voisinage de la surface de celle-ci d'une manière fournissant un verrouillage de forme de sorte que simplement une région partielle desdites particules fasse saillie de ladite couche intérieure, et dans lequel la couche de matière plastique ainsi préparée est recouverte d'une couche fonctionnelle extérieure, résistant à l'usure, électriquement isolante dans laquelle les régions partielles de particules faisant saillie de ladite couche de matière plastique sont intégrées.

2. Procédé selon la revendication 1, dans lequel les particules sont projetées dans la matrice de matériau de la couche de matière plastique ainsi chauffée au voisinage de la surface de celle-ci.

3. Procédé selon la revendication 1 ou 2, dans lequel, à une étape d'une opération de pulvérisation thermique pour produire la couche fonctionnelle, les premières particules de poudre sont projetées dans la matrice de matériau de la couche de matière plastique chauffée au voisinage de la surface de celle-ci d'une manière telle qu'une région partielle de celles-ci fait encore saillie de ladite couche de matière plastique, et dans lequel, au cours de l'opération de pulvérisation, en outre, les particules de poudre faisant saillie sont amenées à être liées à des particules de poudre subséquentes formant ladite couche fonctionnelle.

4. Procédé selon l'une quelconque des revendications précédentes, dans lequel ladite couche fonctionnelle extérieure est produite en une épaisseur de 0,05 mm à 3,0 mm, et de préférence en une épaisseur d'environ 0,5 mm.

5. Procédé pour produire un cylindre corona comprenant un corps de base cylindrique et un élément de recouvrement de cylindre en un matériau diélectrique, dans lequel une couche de matière thermoplastique est appliquée sur la surface extérieure du corps de base, dans lequel la couche de matière plastique est chauffée à une viscosité similaire à celle du miel, dans lequel des particules de matière solide ayant des caractéristiques d'isolement électrique sont dispersées dans la matrice de matériau de la couche de matière plastique ainsi chauffée au voisinage de la surface de celle-ci, et dans lequel une surface dure résistant à l'usure et à la corrosion est produite en meulant ensuite l'élément de recouvrement en matière thermoplastique dans lequel des particules de matière solide sont dispersées au voisinage de sa surface.

6. Procédé selon la revendication 5, dans lequel les particules de matière solide sont dispersées dans la matrice de matériau de la couche de matière plastique ainsi chauffée au voisinage de la surface de celle-ci au moyen d'un système de sablage et de calandrage.

7. Procédé selon l'une quelconque des revendications précédentes, dans lequel ladite couche de matière plastique est appliquée sur le corps de base du cylindre par un processus à lit fluidisé ou un processus de pulvérisation thermique.

8. Procédé selon l'une quelconque des revendications précédentes, dans lequel ladite couche de matière plastique est appliquée en une épaisseur de 0,5 mm à 4 mm.

9. Procédé selon l'une quelconque des revendications précédentes, dans lequel la surface de l'élément de recouvrement de cylindre est meulée ou polie avec une rugosité de surface de 0,5 µm < Rz < 500 µm, particulièrement une rugosité de surface Rz de 1,5 µm à 20 µm.

10. Cylindre corona comprenant un corps de base cylindrique et un élément de recouvrement de cylindre en un matériau diélectrique, **caractérisé en ce que** l'élément de recouvrement de cylindre comprend une couche de matière thermoplastique appliquée à la surface extérieure du corps de base, dans lequel des particules de poudre solide ayant des caractéristiques d'isolement électrique sont intégrées dans la matrice de matériau de ladite couche au voisinage de la surface de celle-ci d'une manière fournissant un verrouillage de forme de sorte que simplement une région partielle desdites particules fasse saillie de ladite couche intérieure, et **en ce qu'**une couche fonctionnelle extérieure dure résistant à l'usure et à la corrosion est formée du côté extérieur de ladite couche de matière thermoplastique, dans laquelle les régions partielles de particules faisant saillie de ladite couche de matière plastique sont intégrées, ladite couche fonctionnelle extérieure dure résistant à l'usure et à la corrosion ayant également des caractéristiques d'isolement électrique.

11. Cylindre corona selon la revendication 10, **caractérisé en ce que** la couche fonctionnelle consiste en une céramique d'oxyde, en particulier l'Al₂O₃, le Cr₂O₃, le SiO₂, le ZrO₂ ou la mullite ou un mélange de deux desdits matériaux ou plus.

12. Cylindre corona selon la revendication 10 ou 11, **caractérisé en ce que** la matière thermoplastique a une résistance spécifique d'au moins 10¹² Ω x m et/ou consiste en du polyamide.

13. Cylindre corona selon l'une quelconque des revendications 10 à 12, **caractérisé en ce que** les particules intégrées dans la matrice de matériau de la couche de matière plastique au voisinage de la surface de celle-ci consiste en le même matériau que celui de la couche fonctionnelle.

14. Cylindre corona selon l'une quelconque des revendications 10 à 13, **caractérisé en ce que** la couche de matière plastique a une épaisseur de 0,5 mm à 4 mm et/ou la couche fonctionnelle a une épaisseur de 0,05 mm à 3,0 mm et de préférence d'environ 0,5 mm.

15. Cylindre corona selon l'une quelconque des revendications 10 à 14, **caractérisé en ce que** la surface de l'élément de recouvrement de cylindre a une rugosité de surface de 0,5 µm < Rz < 500 µm, en particulier une rugosité de surface Rz de 1,5 µm à 20 µm.
